

[54] **IMPACT RESISTANT COATINGS FOR NICKEL-BASE AND COBALT-BASE SUPERALLOYS AND THE LIKE**[75] Inventors: **Richard J. Stueber, Suffern, N.Y.; Stanley J. Klach, Riverdale, N.J.**[73] Assignee: **Chromalloy American Corporation, Orangeburg, N.Y.**[22] Filed: **Aug. 19, 1970**[21] Appl. No.: **65,147**[52] U.S. Cl. .... **117/107.2 P**, 117/131, 29/197[51] Int. Cl. .... **C23c 9/02**[58] Field of Search ..... **117/107.2**[56] **References Cited**

## UNITED STATES PATENTS

3,544,348 12/1970 Boone et al. .... **117/107.2 P**

|           |        |                      |             |
|-----------|--------|----------------------|-------------|
| 3,257,230 | 6/1966 | Wachtell et al. .... | 117/107.2   |
| 3,073,015 | 1/1963 | Wachtell et al. .... | 117/107.2 X |
| 3,096,205 | 7/1963 | De Guisto ....       | 117/107.2   |
| 3,436,249 | 4/1969 | Lambert et al. ....  | 117/130 X   |

Primary Examiner—Ralph S. Kendall

Attorney—Sandoe, Hopgood and Calimafde

[57]

**ABSTRACT**

In the production of impact and oxidation resistant nickel-base metal coatings on heat resistant superalloys by pack aluminizing in which nickel aluminide is formed to provide the protective coating, markedly improved ductile coatings are produced of high impact resistance by controlling the amount of aluminum in the pack which also contains about 5 to 40 percent by weight of chromium, the amount of aluminum not exceeding 3 percent by weight of the pack.

3 Claims, 1 Drawing Figure





IMPACT RESISTANCE (IN-LBS)

INVENTORS  
 RICHARD J. STUEBER  
 STANLEY J. KLACH  
 BY

Sandoe, Hopgood & Calimafde  
 ATTORNEYS

# IMPACT RESISTANT COATINGS FOR NICKEL-BASE AND COBALT-BASE SUPERALLOYS AND THE LIKE

This invention relates to the pack-aluminizing of heat resistant superalloy substrates and, in particular, to a method of producing a hot corrosion resistant metal coating on nickel-base superalloys, wherein the aluminized coating is characterized by improved resistance to impact at ambient and elevated temperatures.

## BACKGROUND OF THE INVENTION

Metallurgical developments in recent years have indicated the necessity of using high nickel and high cobalt heat resistant alloys, e.g. superalloys having desirable physical properties for various high temperature applications, such as, for example, the manufacture of rotor blades and stator vanes for high temperature gas turbines where operation without failure is desired of the part, such as during prolonged exposure to temperatures well above 1,500°F and even substantially above the temperature range at which failure or diminution of the strength characteristics may be expected of even high temperature austenitic or nickel chromium steel.

The use of superalloys by themselves with nothing more have not always provided the necessary resistance to hot corrosion damage at such elevated temperatures. Thus, corrosion resistant coatings have been resorted to as one means of further augmenting the resistance of the substrate to high temperature corrosion, particularly on complex shaped components used in contemporary jet engines where handling and gauging damage have been known to cause premature failure of protective coatings which tend to be brittle in nature.

A wide variety of different processes and techniques are known for producing a diffusion coating or layer into or on the surface of metal articles. Some of these well-known techniques (and those generally of the character to which this invention particularly relates) involved embedding the article to be coated (or otherwise covering the surface thereof) in powdered coating pack including a powdered source of the coating material (with or without admixture with powdered inert filler) and a vaporizable halogen carrier ingredient (such as a heat-volatile halide), and heating the thus embedded article and pack in a sealed retort (or other controlled and generally non-oxidizing atmosphere) to an elevated temperature at which the carrier material vaporizes and/or otherwise reacts with or functions as a carrier for transporting the coating material from or through the powdered pack to the surface of the article to be coated for diffusion or other reaction therat.

Generally speaking, the various chemical reactions involved (e.g., between the carrier and the coating material, and the metal or other components of the article to be coated, among whatever ingredients are in the pack, between coating material and whatever intermetallics or alloys may have already been formed at or in the surface of the article being coated, etc.) occur more or less simultaneously during the heating treatment and are mostly of a reversible nature, so that the net result of the coating step and the chemical reactions therein involved may depend predominantly upon

the various equilibria achieved. That is, as will be understood, under certain temperature conditions and with certain reactive carrier materials, ingredients in the coating pack may be inclined to combine with each other at the same time (and, perhaps, even at the same rate) as one or another thereof may diffuse into the surface of the metal article; while (if the equilibrium conditions are appropriate) some portion of the metal from the article itself, or one of another component thereof, may also "diffuse" out of the article and into the pack ingredients.

## RELATED U.S. PATENT

In U.S. Pat. No. 3,257,230 assigned to the same assignee, it is stated that aluminum diffusion into the surface of a predominantly nickel-containing article may be productive of a variety of different nickel aluminides, with the particular one formed being perhaps a function of the proportion of aluminum carried to the article surface or diffused therein at the particular operating temperature. If the particular aluminide desired is one containing less than the maximum amount of aluminum, formation thereof may not occur if aluminum from the pack be too rapidly presented to or available in the article surface. If the treatment is maintained at a sufficiently high temperature and prolonged to achieve a desired thickness of coating layer, too rapid transfer of aluminum from the pack to the surface of the article (or too slow diffusion from the surface on inwardly of the article) may occur to form a lower melting high-aluminum aluminide rather than the one desired.

It was discovered that the foregoing could be avoided by including a portion of a buffering material, such as chromium, in the pack to form with the aluminum therein a preliminary intermetallic, the diffusion of which into the surface of the article can only occur at a diminished rate (or, perhaps, cannot occur at all) at the desired treating temperatures, the availability or transfer of the aluminum component in the pack for diffusion into the surface of the article is readily inhibited or controlled so that the temperature levels or other thermodynamic conditions necessary to break down the preliminary chromium aluminide sufficiently for aluminum to be diffused will produce the desired conditions for the formation of the particular nickel aluminide desired in the surface of the article.

Utilizing an inhibiting or rate controlling component such as chromium in an aluminum pack for preliminary formation therein of a chromium aluminide has been found to produce satisfactory results in that temperatures high enough to break down the chromium aluminide for diffusion coating of aluminum are at levels where the desired particular nickel aluminide forms in the surface of a nickel-containing alloy.

It has been found according to the aforementioned patent that in the broad sense aluminum coatings are obtainable from a chromium-containing pack containing about 3 to 20 percent by weight of aluminum, the pack preferably also containing an inert diluent, such as powdered refractory oxides, e.g. alumina, magnesia, calcia, silica, zirconia and the like. It was noted that the ratio of chromium to aluminum in the pack may range up to 8 and, more preferably, from about 0.5 to 4.6 (e.g. 2 to 4). A composition found particularly satisfac-

tory for commercial use is one containing by weight 69% alumina as the inert diluent, 22% chromium, 8% aluminum and 1% ammonium fluoride, with the coating layer or casing depths of the order of about 0.0019 inch to 0.0022 inch. In producing the coating, the pack is enclosed in a sealed container and heated at between 1,800° to 2,100°F for 4 to 20 hours, with the temperature and time ranging more broadly from about 1,400° to 2,200°F for 1/4 to 40 hours. Severe oxidation testing at 2,000°F in an oxidizing atmosphere provided in a standard testing furnace indicated no failure of any of the coated parts in over 85 hours of testing treatment.

While markedly improved resistance to oxidation at elevated operating temperatures was obtainable due to the nickel aluminide formed in the coating by the foregoing process, the coatings did not have the desired resistance to impact. Care had to be exercised in the handling of coated parts during assembly-line production. Impact-resistant coatings are required on current turbine engine hardware of complex geometries to insure that protection of the base metal is not lost as a result of chipping or spalling due to in-shop handling on the production line. Thus, a diffusion heat treatment is generally required to improve the impact resistance of the coating. However, even then failure might occur during handling of the coated part prior to heat treatment.

#### OBJECTS OF THE INVENTION

It is thus an object of this invention to provide a pack-aluminizing process for producing ductile, hot corrosion resistant nickel aluminide coatings which do not require a diffusion heat treatment for improving the impact resistance thereof.

Another object is to provide a pack aluminizing process for producing a nickel aluminide coating of uniform thickness capable of sustaining severe plastic deformation, such as that resulting from impact without cracking or spalling.

Still another object is to provide a pack aluminizing process for producing a ductile nickel aluminide coating which will permit the base metal substrate to be strained during use into its plastic range while undergoing heavy loading or thermal stress without the coating cracking or spalling.

These and other objects will more clearly appear from the following disclosure, the appended claims and the accompanying drawing which is a graph illustrating the markedly improved resistance to impact obtained with the novel method of the invention.

#### BRIEF SUMMARY OF THE INVENTION

Stating it broadly, the invention resides in a method of pack aluminizing nickel-base heat resistant alloys, such as superalloys, wherein an article of the alloy is embedded in a cementation pack containing chromium metal, an inert diluent (e.g. alumina), and an amount of aluminum metal sufficient to effect the diffusion coating thereof at an elevated diffusion temperature into the surface of the article by means of a vaporizable halogen transport agent or a carrier, the improvement residing in controlling the amount of aluminum in the pack over the range of about one-eighth to not more than 5 percent by weight of the pack. By maintaining the aluminum over the foregoing range and, more advantageously, over the range of about 1/2 to 2.5 percent, a ductile protective metal coating is assured characterized by improved resistance to impact at room and elevated temperatures.

The coating produced by the aforementioned process has a uniform thickness and can sustain severe plastic deformation, such as that resulting from impact, without cracking or spalling in such a way as to affect adversely the sulfidation and oxidation resistance of the coating. The ductility of coatings produced in accordance with the invention permits the base metal substrate to be strained into its plastic range while undergoing heavy loading or thermal stress with the result that the coating does not crack or spall.

A wide range of nickel-base alloys can be coated using the foregoing method. A typical alloy composition range is one containing by weight of up to about 30% Cr, e.g. 5% to 30% Cr, up to about 20% of a metal from the group consisting of Mo and W, up to about 10% of a metal from the group consisting of Cb and Ta, up to about 1% C (preferably up to about 0.5%), up to about 10% by weight of a metal from the group consisting of Ti and Al, the total amount of Ti and Al not exceeding about 12%, up to about 20% Fe, up to about 2% Mn, up to about 2% Si, up to about 0.2% B, up to about 1% Zr, up to about 2% Hf, and the balance at least about 45% by weight of nickel.

Examples of known alloys falling within the aforementioned range are nickel-base alloys referred to by designations Mar-M-246, IN-738, IN-792 Udimet 500, Mar-M-432, In-713, Mar-M-200, B-1900, TRW-6A, IN-600 and Udimet 700, and cobalt-base alloys, such as WI-52 and Mar-M-509. Compositions of the foregoing illustrative alloys are given in Table 1 as follows:

TABLE I

| Alloy designation | Chemical composition, weight percent |      |      |       |       |       |       |       |       |       |        |         |        |
|-------------------|--------------------------------------|------|------|-------|-------|-------|-------|-------|-------|-------|--------|---------|--------|
|                   | C                                    | Cr   | Ni   | Co    | Mo    | W     | Cb    | Fe    | Ti    | Al    | B      | Zr      | Others |
| IN-738-----       | 0.13                                 | 15.9 | Bal. | 8.5   | 1.8   | 2.6   | 0.9   | 0.1   | 3.5   | 3.4   | 0.011  | 0.11    | 1.9 Ta |
| IN-792-----       | 0.21                                 | 12.7 | Bal. | 9.0   | 2.0   | 3.9   | ----- | ----- | 4.2   | 3.2   | 0.02   | 0.1     | 3.9 Ta |
| IN-713C-----      | 0.12                                 | 12.5 | Bal. | 4.2   | ----- | 2.0   | ----- | 0.8   | 6.1   | 0.01  | 0.10   | -----   |        |
| IN-600-----       | 0.04                                 | 15.8 | Bal. | ----- | ----- | 7.2   | ----- | ----- | ----- | ----- | 0.2 Mn | 0.2 Si  |        |
| Udimet 500-----   | 0.08                                 | 18.0 | Bal. | 18.5  | 4.0   | ----- | ----- | 2.9   | 2.9   | 0.006 | 0.05   | -----   |        |
| Udimet 700-----   | 0.08                                 | 15.0 | Bal. | 18.5  | 5.2   | ----- | ----- | 3.5   | 4.3   | 0.03  | -----  | -----   |        |
| Mar-M-200-----    | 0.15                                 | 9.0  | Bal. | 10.0  | 7.8   | 12.5  | 1.0   | ----- | 2.0   | 5.0   | 0.015  | 0.05    | -----  |
| Mar-M-246-----    | 0.15                                 | 9.0  | Bal. | 10.0  | 2.5   | 10.0  | ----- | ----- | 1.5   | 5.5   | 0.015  | 0.05    | 1.5 Ta |
| Mar-M-432-----    | 0.15                                 | 15.4 | Bal. | 19.7  | ----- | 3.0   | 1.8   | ----- | 4.4   | 2.9   | 0.013  | 0.03    | 2.2 Ta |
| B-1900-----       | 0.10                                 | 8.0  | Bal. | 10.0  | 6.0   | ----- | ----- | ----- | 1.0   | 6.0   | 0.015  | 0.10    | 4.0 Ta |
| TRW-6A-----       | 0.13                                 | 6.1  | Bal. | 7.5   | 2.0   | 5.8   | 0.5   | ----- | 1.0   | 5.4   | 0.02   | 0.13    | 9.0 Ta |
| WI-52-----        | 0.45                                 | 21.0 | Bal. | 11.0  | 11.0  | 2.0   | 2.0   | ----- | ----- | ----- | 0.4 Hf | 0.14 Re |        |
| Mar-M-509-----    | 0.6                                  | 21.0 | 10.0 | Bal.  | ----- | 7.0   | ----- | 1.5   | 0.2   | ----- | 0.01   | 0.5     | 3.5 Ta |
|                   |                                      |      |      |       |       |       |       |       |       |       | 0.1 Mn | 0.1 Si  |        |

In carrying out the pack cementation process, a set of double nested retorts is used in which the inner and outer retorts are glass sealed to inhibit the entry of air during the coating process. However, single retorts may be used as well. The pack is freshly prepared and then prereacted by heating the pack to a temperature of, for example, 1,800° to 2,200°F for about 1 to 20 hours, the pre-reacted powder being then screened and used as the pack into which the article to be coated is then embedded. The pack composition may range by weight from about 5 to 40 percent chromium, or 10 to 30% chromium, about one-eighth to not more than 5% aluminum, a small but effective amount of a halogen material energizer (e.g. from about one-eighth to 1 or 2 percent) and the balance a diluent material, e.g. such refractory oxides as alumina, zirconia, calcia, silica, and the like.

#### DETAILS OF THE INVENTION

Typical powder materials employed in making up the pack are given by way of example as follows:

| Pack Constituent    | Function      | Particle Size |
|---------------------|---------------|---------------|
| Aluminum            | Coating Metal | -325 mesh     |
| Chromium            | Buffer        | -100 mesh     |
| Aluminum Oxide      | Inert Filler  | -325 mesh     |
| Ammonium Bifluoride | Energizer     | -80 mesh      |

Examples of other energizers are  $\text{NH}_4\text{I}$ ,  $\text{NH}_4\text{Br}$ ,  $\text{NH}_4\text{Cl}$ , and the like. Broadly speaking, the diffusion coating treatment is carried out at a temperature of about 1,400° to 2,200°F for about  $\frac{1}{4}$  to 40 hours. A more preferred range is 1,750° to 2,050°F for about 10 to 30 hours. A pack cementation treatment found particularly advantageous in coating alloys of Table 1 is 1,900°F for about 25 hours at temperature, using a blended powder pack composition containing 20% chromium, 2% aluminum, about  $\frac{1}{4}\%$  ammonium bifluoride and the balance essentially alumina.

In determining the impact resistance of a particular coating, a drop weight test is employed in which a metal weight (e.g. a half-pound weight) with a projection or indenter having a 0.065 inch radius at its impact end is dropped upon a coated test piece from various heights measured in inches, the impact value being determined in inch pounds at the point where the coating fails by cracking or spalling. Alloys coated from a pack containing by weight 20% chromium, 3% aluminum,  $\frac{1}{4}\%$  ammonium bifluoride and the balance essentially alumina resulted in impact values (ductile coating) of over 17 inch pounds (high impact resistant), while the same pack containing 8% by weight of aluminum resulted in inferior impact values (brittle coating) as low as 3 inch pounds.

The improved ductility of the coating provided by the invention enables the coating to deform as the base metal substrate is strained due to applied load or thermal stress arising in the environment of use, such as air-

foils, in jet engines. This ability of the coating to deform with fracture with applied stress, such as might arise from thermal shock, protects the base metal against catastrophic oxidation or hot corrosion. In the case of the more brittle nickel or cobalt aluminide coatings produced outside the invention, load-induced strain of the base metal in the elastic range resulted in severe cracking of the coating.

As illustrative of the preferred embodiment of the invention, the following example is given.

#### Example 1

A series of pack cementation compositions was tested in which the aluminum in the pack was varied from about one-eighth to 8 percent by weight with the 20 chromium level at about 20 percent. The pack also contained about  $\frac{1}{4}\%$   $\text{NH}_4\text{FHF}$  and the balance alumina. The tests were carried out on a series of commercial nickel-base alloys, the compositions of which are given in Table 1. Test pieces of each alloy were embedded in the pack in a sealed retort which pack had first been pre-reacted (as described hereinbefore) and the coating step carried out at 1,900°F for 25 hours. Following the coating, the test pieces were brushed clean and then subjected to the impact test described hereinbefore. The resulting coatings varied in thickness from about 1.2 to 5 mils (0.0012 to 0.005 inch) and seemed to relate directly to the amount of aluminum powder in the pack. Thus, the thinnest coating was obtained at the lower range, while the 5 mil thickness was obtained with the pack containing 8% aluminum. The coatings which exhibited optimum impact values of over 17 inch pounds and which were ductile were obtained in pack compositions containing not more than 5 percent aluminum. At aluminum contents in the pack of over 5 percent, that is, over 6, 7 and up to 8 percent, the coatings were brittle and exhibited impact values as low as 3 inch pounds. The results obtained in the aforementioned tests are given in Table 2.

To determine whether the ductility of the coating was a function of the case depth of the coating per se, the following experiment was performed. The impact specimen was coated in a powder mixture containing 20% Cr, 3% Al,  $\frac{1}{4}\%$   $\text{NH}_4\text{FHF}$  and the balance  $\text{Al}_2\text{O}_3$ , and the specimen removed from the powder pack and impact tested. The impact value was greater than 17 inch pounds. The same specimen was subsequently coated again in a powder mixture of the same composition, removed and impact tested. The result was an impact value of greater than 17 inch pounds. Metallographic inspection of the coating on this specimen revealed a case depth of 5.1 mils (0.0051 inch).

The unexpected result obtained with packs containing one-eighth to not more than 5% aluminum was not recognized in U.S. Pat. No. 3,257,230. In fact, the patent states at column 11, lines 13 to 17, that, for its purposes, a pack composition of 69% alumina, 22% chromium, 8% aluminum and 1% ammonium fluoride was satisfactory. Thus, the patent is not aware that ductile coatings can be obtained provided that the aluminum in the pack does not exceed 5 percent.

TABLE 2

[Effect of pack compositions on impact ductility and coating thickness of aluminide type coatings on nickel base superalloys]

| Alloy      | Pack Composition (w/o Al) (20 Cr-X Al-1/4 NH <sub>4</sub> FHF-Bal. Al <sub>2</sub> O <sub>3</sub> ) |       |       |       |       |       |       |         |
|------------|-----------------------------------------------------------------------------------------------------|-------|-------|-------|-------|-------|-------|---------|
|            | 1/8                                                                                                 | 1/2   | 3/4   | 1.5   | 2     | 3     | 5     | 8       |
| Mar-M-246  | D/2.0*                                                                                              | D/2.5 | D/2.8 | D/2.6 | D/2.5 | D/3.0 | D/3.0 | B/5.0** |
| Mar-M-200  | D/2.5                                                                                               | D/2.5 | D/2.5 | D/2.5 | D/2.5 | D/3.0 | D/3.0 | B/5.0   |
| Mar-M-432  |                                                                                                     |       | D/1.5 | D/2.0 | D/1.5 | D/1.8 | D/2.0 | B/4.5   |
| IN-738     | D/2.0                                                                                               | D/3.5 | D/2.5 | D/2.5 | D/3.0 | D/2.5 | D/3.5 |         |
| IN-792     | D/1.5                                                                                               | D/2.5 | D/2.3 | D/2.5 | D/2.5 | D/2.5 | D/2.5 |         |
| IN-713     | D/2.5                                                                                               | D/2.5 | D/2.0 | D/2.2 | D/3.5 | D/3.5 | D/3.5 | B/5.0   |
| Udimet 500 | D/1.5                                                                                               | D/1.9 | D/1.8 | D/2.0 | D/2.0 | D/2.0 | D/2.8 |         |
| B-1900     | D/2.0                                                                                               | D/2.5 | D/2.3 | D/1.8 | D/3.0 | D/3.0 | D/3.0 | B/5.0   |
| TRW-6A     | D/1.2                                                                                               | D/1.5 | D/1.5 | D/2.0 | D/2.0 | D/2.5 | D/2.5 | B/5.0   |

\*D=Ductile impact values greater than 17 inch pounds.

\*\*B=Brittle impact values less than 17 inch pounds.

NOTE.—Coating thickness is given in mils (one mil=0.001").

Similar tests were conducted using a pack containing 10% chromium, 1/4% NH<sub>4</sub>FHF, from 1 to 3% aluminum and the balance alumina. While only half as much chromium was used in the pack, good ductile coatings were obtained exhibiting optimum impact values of

The values of over 17 inch pounds reported for the tests on coatings within the invention means that no spalling or cracking occurred when the half-pound weight was dropped from a height of 34 inches ( $\frac{1}{2} \times 34 = 17$  inch pounds), the limit of the apparatus. However, at an aluminum composition in the pack of 8 percent, the coating was very brittle and gave a reading of 3 inch pounds, thus indicating that the coatings of the invention are over five times better insofar as impact resistance is concerned, using the drop test as the criterion.

Using a one-and-one-half pound weight (1 1/2 lb) corresponding to a total impact from a maximum height of 34 inches of 51 inch pounds ( $1\frac{1}{2} \times 34 = 51$ ), the curve shown in the attached drawing was obtained on the coated alloy designated as Mar-M-246 (note Table 1). The pack was varied from 1/8% aluminum up to 8% aluminum, the pack also containing 20% chromium, 1/4% of NH<sub>4</sub>FHF and the balance alumina. The aluminizing was carried out at 1,900°F for 25 hours. Between about 1/8 to 2 1/2 percent aluminum in the pack (especially between about 1/2 to 2 1/2%), failure at impact (that is, cracking of the coating) began at the relatively high level of about 35 inch pounds (optimum impact resistance) with the impact value beginning to fall off at above 2 1/2% aluminum and thereafter at a fairly rapid rate at just below 5% aluminum pack concentration. From below 5% aluminum to about 6 percent and 7% aluminum pack concentration, the falling off in impact resistance is sharp and reaches a very low level of between 2 1/2 to 3 inch pounds at 8% aluminum concentration. Thus, below 5% aluminum concentration, the coating has good ductility and exhibits relatively high impact values, the optimum impact values being achieved about 2 1/2% aluminum concentration and below, that is, advantageously from about 1/2 to 2 1/2% aluminum concentration.

Room temperature tensile testing of a coated IN-713C alloy (coated in a pack of 20% Cr-3% Al-1/4% NH<sub>4</sub>FHF and Al<sub>2</sub>O<sub>3</sub> the balance), showed that no cracking occurred when the alloy was loaded and strained throughout the elastic range when viewed under a microscope at a magnification of 500 times. It was found that the coated alloy could withstand a total strain, i.e. plastic deformation, of up to 0.3%. Additional testing has shown that the coating produced in

accordance with the invention exhibited good oxidation resistance in excess of 400 hours at 2,000°F. Good sulfidation and hot corrosion protection were indicated at the same temperature far in excess of 100 hours.

The pack composition may range by weight broadly from about 5 percent to 40 percent chromium, about 1/8% to not more than 5% aluminum, about 1/8 to 1 or 2% halide energizer (e.g. about 1/4% NH<sub>4</sub>FHF) and the balance essentially a refractory oxide diluent, e.g. alumina. Within the foregoing ranges, the chromium may be controlled from about 7 to 30 percent and the aluminum from about 1/2 percent to 2 1/2%. We have found it advantageous in working over the foregoing ranges to employ a chromium to aluminum ratio of about 4:1 to 160:1 and, more advantageously, about 8:1 to 100:1.

Although the present invention has been described in conjunction with preferred embodiments, it is to be understood that modifications and variations may be resorted to without departing from the spirit and scope of the invention as those skilled in the art will readily understand. Such modifications and variations are considered to be within the purview and scope of the invention and the appended claims.

What is claimed is:

1. A method of producing aluminized coatings on nickel-base heat resistant alloys characterized by markedly improved ductility under impact which comprises:

providing said alloy having a composition containing by weight, up to about 30% Cr, up to about 20% of a metal from the group consisting of Mo and W, up to about 10% of a metal from the group consisting of Cb and Ta, up to about 1% C, up to about 10% by weight of a metal from the group consisting of Ti and Al, the total amount of Ti and Al not exceeding about 12%, up to about 20% Fe, up to about 2% Mn, up to about 2% Si, up to about 0.2% B, up to about 1% Zr, up to about 2% Hf, and the balance at least about 45% by weight of nickel; preparing an aluminum-containing pack consisting essentially by weight of about 5 to 40% chromium, an effective amount of aluminum not exceeding 3 percent, a small but effective amount of a halide energizer, and the balance an inert diluent, prereacting said pack by heating said pack at a temperature ranging from about 1,800°F to 2,200°F, embedding a nickel-base heat resistant alloy in said prereacted pack,

and carrying out said method at an elevated aluminizing temperature with the amount of aluminum in said pack less than 3 percent, the ratio of chromium to aluminum in said pack being in ex-

cess of 4:1, whereby a coating containing nickel aluminide and having markedly improved ductility is obtained.

2. The method of claim 1, wherein the chromium content of said pack ranges by weight from about 10 to 30%, the aluminum content ranging from about ½% to

2½% and the inert diluent is a refractory oxide.

3. The method of claim 1, wherein the ratio of chromium to aluminum in the pack ranges from above 4:1 to 160:1.

\* \* \* \* \*